

Feb. 22, 1949.

J. KNIVETON

2,462,202

## HEAT TREATING

Filed Jan. 29, 1944

2 Sheets-Sheet 1

Fig. 1.



INVENTOR

**WITNESS**

F. J. Hartman.

BY *El Fernander*  
*his ATTORNEY*

Feb. 22, 1949.

J. KNIVETON

2,462,202

## HEAT TREATING

Filed Jan. 29, 1944

2 Sheets-Sheet 2

Fig. 2.



Fig. 3.



INVENTOR

WITNESS

F. J. Hartman.

James Knickerbocker  
BY W. Fernando  
his ATTORNEY

## UNITED STATES PATENT OFFICE

2,462,202

## HEAT TREATING

James Kniveton, Wyncote, Pa., assignor to Selas Corporation of America, a corporation of Pennsylvania

Application January 29, 1944, Serial No. 520,271

7 Claims. (Cl. 148—13)

1

My invention relates to the art of heat treating strips, sheets, wires and the like which are passed continuously through a furnace.

The rate at which work of the above-described type can be heat treated in the usual type of furnace is dependent upon the rate at which heat is transferred to the work and the size of the work passed through a particular length of heating chamber of a furnace. Thus, in a heat treating furnace in which annealing is effected, the work passes into the charging end of the furnace at room temperature and during its travel through the furnace it must be heated to the annealing temperature. When this annealing temperature is reached, only a portion of the length of the heating chamber is utilized to maintain and hold the work at this annealing temperature.

In accordance with my invention, in order to increase the rate at which strips, sheets, wires and the like can be heat treated, it is proposed to provide a high temperature heating chamber immediately ahead of the charging end of the heat treating furnace. This high temperature heating chamber, which may be referred to as a pre-heating chamber, is of relatively high heat capacity and effective to heat saturate the work rapidly substantially to the desired elevated temperature. By heat saturating the work it is meant that either complete heat saturation of successive portions of the work may be effected in the high temperature heating chamber, or such surface heat saturation may be effected that the inner core of the work will be brought up to the desired high temperature for the heat treating operation to be effected in the heat treating furnace.

In annealing, for example, the advantage of rapidly heating the work to a definite elevated temperature in the preheating chamber, before the work enters the chamber of the annealing furnace, is that the furnace substantially in its entirety may serve as a holding and stabilizing chamber. In other words, the work can be held and maintained at the desired annealing temperature substantially during its entire travel through the annealing furnace, so that a tremendous increase in the rate at which work is annealed can be effected. In this way the production rate of existing annealing furnaces can be stepped up to a substantial degree. Further, such faster speeds at which work can be annealed may be effected without operating the annealing furnace at excessive furnace temperatures which would burn the work when the work stops moving in the annealing furnace.

2

An object of my invention is, therefore, to provide an improvement for increasing the rate at which work passing continuously through a furnace can be heat treated in which the surface of the work or the work in its entirety is rapidly heat saturated to a desired elevated temperature immediately before the work enters the charging end of the heat treating furnace.

Another object of my invention is to heat work rapidly to a high temperature for a heat treating operation just before entering the charging end of the heat treating furnace by a high heat capacity heating chamber capable of producing a relatively high thermal head.

15 A further object of my invention is to provide such a high heat capacity heating chamber immediately ahead of the charging end of a heat treating furnace, such as an annealing furnace, for example, which may be readily rendered ineffective to heat the work sufficiently to burn it, in the event of work stoppage in the heating chamber.

20 The novel features which I believe to be characteristic of my invention are set forth with particularity in the claims. The invention itself, however, both as to organization and method, together with further objects and advantages thereof, will be better understood by reference to the following description taken in connection with the accompanying drawings of which Fig. 1 more or less diagrammatically illustrates a sectional view of annealing apparatus embodying the invention; Fig. 2 is an enlarged fragmentary view of the preheating chamber shown in Fig. 1, 25 to illustrate the invention more clearly; Fig. 3 is a top plan view of the preheating chamber shown in Fig. 2; and Fig. 4 is a sectional view 30 more or less diagrammatically illustrating a modification of the invention.

35 In the drawings my invention has been shown in connection with the annealing of wires, although it is to be understood that the invention is equally applicable to the annealing of strips, sheets and the like and to other heat treating operations. Referring more particularly to Fig. 1, a wire 10 to be annealed is unwound from a coil 11 and passed over a guide pulley 12. From the guide pulley 12 the wire 10 passes downwardly through a preheater 14 and an annealing furnace 15 into a quench tank 16 containing a body of quenching liquid 17, such as water, for example. The wire 10 then passes over a guide pulley 18 in quench tank 16 and upwardly through a drying unit 19. From the drying unit 19 the wire 10 passes over a guide pulley 20 and

thence rewound at coil 21. Although only a single strand of wire 10 is shown in Figs. 1 and 2, it should be understood that a plurality of strands of wire 10 may be passed simultaneously through heating chamber 14, furnace 15, quench tank 16, and drying unit 18. In Fig. 3 a plurality of such strands of wire 10 are shown passing through heating chamber 14.

The annealing furnace 15 illustrated is of a gas fired type having vertical walls 22 and a roof 23 formed of suitable refractory material. The vertical walls 22 and roof 23 are disposed within a framework or outer shell 24 supported by a foundation 24a on a supporting surface. The roof 23 constitutes the charging end of the furnace 15 and is formed with an opening 25 into which the wire 10 passes for the annealing operation. A plurality of hinged flaps 26 may be provided at the top of the shell 24, in the immediate vicinity of opening 25, to form a narrow space through which the wires 10 may pass into the furnace 15. A downwardly depending hollow skirt 27 is secured to the lower end of furnace 15 and extends into the quench tank 16 below the liquid level therein to seal the lower end of the furnace.

A plurality of burners 28 are mounted and incorporated in the side walls 22 of furnace 15. The burners 28 are arranged at different elevations and disposed alongside of each other in a plurality of rows, the number of burners and distribution being such that the desired heating is effected of the wire 10 passing through the furnace chamber 29.

The burners 28 are mounted in and form a part of the side walls 22. Each burner 28 comprises a molded block of ceramic material having a central passage within which is disposed a burner tube or sleeve 30. The outer ends of sleeves 30 are connected to manifolds 31 to which a gas mixture is delivered through conduits 31a from a suitable source of supply. Suitable valves 32 may be provided to control the pressure and rate at which the gas mixture is supplied to the manifolds 31, and the supply of the gas mixture for each burner 28 may be individually controlled by a valve (not shown) operable by a control member 33 disposed at the exterior of the manifold 31.

The gas mixture, which may be a mixture of air and ordinary city gas, is supplied to each of the burners 28 and subdivided into a plurality of gas streams by a distributor or tip 34 fixed to the inner end of the tube or sleeve 29 which terminates at a cup-shaped space 35. A plurality of burner flames are produced and maintained about the peripheral surface of each distributor 34 and project outwardly therefrom into the cup-shaped spaces 35 in which combustion of the gas mixture is effected. The combustion spaces 35 are of such shape and the flames project outwardly at such an angle from the axes of the burners that the flames are closely adjacent and follow the cup-shaped refractory walls to heat the latter to high temperatures approaching incandescence.

The burners 28 are of the kind described and illustrated in Hess Patent No. 2,215,079, granted on June 23, 1942, and assigned to the same assignee as this application. The burners 28 are fully disclosed in the aforementioned Hess patent which may be considered as being incorporated in this application, and, if desired, reference may be had thereto for a detailed description of the burner structure.

By providing the control valves 32 and 33, the gas mixture supplied to the burners 28 may be

accurately controlled so that the desired heating effect may be produced in chamber 29 throughout the height of the chamber. The burners 28 are so constructed that combustion of the gas mixture is substantially completed in the cup-shaped spaces 35, whereby flame impingement on the work is readily avoided. The refractory wall surfaces of the cup-shaped spaces 35 are heated to incandescence and constitute high temperature zones or regions from which heat is radiated to the work. This radiated heat, together with convection heating resulting from the heated products of combustion passing toward the work and downwardly in chamber 29, provides a heating effect which is readily controlled to maintain the wire 10 at the desired annealing temperature during its travel through the furnace 15.

The hinged flaps 26 provide a seal at the top part of furnace 15 so that a positive pressure of the heated products of combustion will be maintained in chamber 29 and prevent flow of air into the furnace chamber. The heated products of combustion pass from the bottom of the furnace chamber 29 through a flue 27a which is connected at its lower end to skirt 27 and may extend upward to a height above the preheater 14.

Since combustion of the gas mixture is substantially completed in the cup-shaped spaces 35, the need for passing the wire 10 through a tube 30 containing a protective atmosphere to protect the wire from burning gases, is avoided. Moreover, the burners 28 may be supplied with a slight excess of gas so that a reducing atmosphere will be maintained in chamber 29. From the furnace 15 the wire 10 passes into the quench tank 16 for the requisite quenching operation when this is necessary.

After being cooled the wire 10 passes through the drying unit 18 comprising an outer shell or framework 36 supported at 37 at one side of the quench tank 16. Within the outer shell 36 are formed walls 38 of refractory material in which are incorporated burners 39 similar to the burners 28 embodied in furnace 15 and described above. The burners 39 are connected to intermediate manifolds 40 which in turn are connected to main manifolds 40a to which are secured flexible conduits 41 through which a gas mixture is delivered from a source of supply. Valves 42 may be provided to control the supply of the gas mixture to the manifolds 40 and individual valves (not shown) may be provided in the conduits leading to the several burners 39 for individually controlling the supply of the gas mixture to each burner 39. The burners 39 are adjusted to produce the desired heating effect in drying chamber 44, and, after the annealed wire has passed through this chamber, the wire 10 passes over the guide pulley 20 and is rewound at coil 21.

In order to provide a controlled temperature in annealing chamber 29, the burners 28 are preferably controlled responsive to the temperature within the chamber. Thus, in the event the rate of movement of the wire decreases, or of complete stoppage of the work, the supply of the gas mixture to the burners 28 may be reduced automatically so that the temperature in chamber 29 will always remain substantially at the desired annealing temperature and not become excessively high to cause burning of the work at slow speeds and when complete stoppage of the work occurs.

In accordance with my invention, in order to increase the rate at which the wire 10 can be annealed in furnace 15, a high temperature heating

chamber 14 is provided immediately ahead of the charging end of the annealing furnace 15. In the embodiment of the invention illustrated in Figs. 1 to 3 inclusive, the preheater or heating chamber 14 comprises two vertical banks of burners 45 in face to face relation at opposite sides of the wire 10 passing therebetween. The vertical banks of burners 45 are movable to an operating position near the wire 10, and are movable rearwardly from the operating position in the event of work stoppage.

As shown in Figs. 2, 3 and 4, the burners 45 are in the form of molded blocks of ceramic material similar to the burners 28 in furnace 15 and are incorporated in and form a part of refractory walls 46. The burners 45 are positioned in the shallow or recessed central parts of the refractory walls 46 disposed within frameworks or outer shells 47 which are U-shaped both in horizontal and vertical sections.

In the illustrated embodiment each bank of burners 45 consists of two horizontal rows of three burners. Each horizontal row of three burners 45 is connected to a horizontally disposed manifold 48, and the horizontal manifolds are in turn connected at intermediate regions to vertically disposed manifolds 49 to which the gas mixture is delivered through flexible conduits 50 from a suitable source of supply. The supply of the gas mixture to each horizontal manifold 48 is controlled by a valve 51, and the supply of the gas mixture to each burner 49 is individually controlled by a valve (not shown) having an adjustable member 52 associated therewith and adjustable at the exterior of the horizontal manifolds, as shown in Fig. 3.

Each bank of burners 45 and associated manifolds 48 and 49 are mounted on a carriage 53 provided with rollers 54 which move in channels or guideways 55 fixed to the top of furnace 15. The guideways 55 are inclined downwardly toward each other and are provided with stops 56 at their lower ends to limit the downward movement of the banks of burners 45 toward the work passing therebetween. The rear of each carriage 53 is connected by cables 57 to a wire 58 which passes over a guide pulley 58a and extends downwardly therefrom. When it is desired to move the banks of burners 45 rearwardly from the operating position shown in Fig. 1, the lower ends of the wires 58 are pulled downwardly, thereby causing the carriages 53 to ride upwardly on the inclined guideways 55.

The preheater or heating chamber 14 is so constructed and arranged that it is capable of heating successive portions of wire 10 rapidly while passing through this chamber. By heating the wire 10 substantially to the desired annealing temperature before the wire enters the charging end of furnace 15, the furnace chamber 29 serves as a holding and stabilizing chamber substantially throughout its entire length and the wire will be substantially at the annealing temperature at the instant it enters the upper end of chamber 29 or within a short interval of time after it enters chamber 29, and then maintained at the annealing temperature throughout substantially its entire travel through the chamber.

The burners 45 are similar to the burners 28 described above and are operated to provide a plurality of zones of radiant heat at temperatures as high as 2600 to 2800° F. These high temperatures are obtained by subdividing the fuel mixture, such as air and ordinary city gas, to produce a plurality of relatively small flames which heat to

incandescence the refractory wall surfaces of the cup-shaped spaces of burners 45. The work passing through the heating chamber 14 is rapidly heated to a high temperature by heat derived from the heated products of combustion passing to the work from the cup-shaped spaces in which combustion of the fuel mixture is substantially completed, and by heat radiated from the incandescent wall surfaces.

In this way an efficient high temperature heating chamber 14 is provided which is capable of operating at a high heat capacity and can rapidly heat wires, strips and sheets and the like to the desired annealing temperature before entering the charging end of the annealing furnace 15. By heating the wire 10 to or substantially to the desired annealing temperature immediately before entering the upper end of furnace 15, the wire 10 can be passed through the annealing furnace at a considerably faster rate than when such preheating is not effected, thereby stepping up the production rate to a substantial degree.

The embodiment just described and illustrated is especially suitable for the bright or clean annealing of work formed of copper, brass, bronze nickel or stainless steel. Although the work may be oxidized when passing through the high temperature heating chamber 14, such work will be deoxidized and cleaned while passing through the furnace chamber 29 by operating the furnace 15 with excess gas to produce a reducing atmosphere in the furnace chamber 29.

The following example of the practice of my invention is given for purposes of illustration only. In a particular installation thirteen (13) gage copper wire has been annealed in an annealing furnace 15 feet long at the rate of 60 feet per minute, the wire being initially heated when first entering the annealing furnace and held and maintained at an annealing temperature of about 1180° F. after being heated to this elevated temperature. When the copper wire is heat saturated to the annealing temperature of about 1180° F. before entering the charging end of the annealing furnace, it is possible to accelerate and step up the rate at which such copper wire is annealed by as much as 30 to 50 per cent. This represents a substantial increase in the rate at which the wire can travel through the annealing furnace and the same bright annealing can be effected at much higher wire speeds.

One of the features contributing to the increased rate of annealing work is due to the provision of relatively high temperature sources of heat provided in heating chamber 14. By providing sources of radiant heat at temperatures varying from 2400 to 2800° F. when an annealing temperature of about 1180° F. is desired in the work itself, as in the example just given, for example, a high thermal head is obtained which results in quick heat penetration in successive portions of the work passing rapidly through the heating chamber 14.

In the event of work stoppage, the supply of gas mixture to all of the burners 39 and 45 may be shut off. This may be effected either manually or automatically responsive to a reduction in the rate of movement of the work. Since the burners 45 in heating chamber 14 operate at relatively high heat capacity and are positioned close to the work passing therethrough, there may be sufficient residual heat to cause burning of the work even after the supply of the gas mixture to the burners 45 is shut off. For this reason provision is made for moving the banks of

7  
burners 45 rearwardly and away from the work when work stoppage does occur or the rate of movement of the wire should decrease.

In Fig. 4 is illustrated a modification of the invention in which the annealing furnace 15a is of a horizontal type having a hearth 9, roof 23a and side walls 22a formed of refractory material and disposed within a framework or outer shell 24a. In the roof 23a are incorporated a plurality of burners 28a similar to the burners 28 shown in Fig. 1 and described above.

The burners 28a are connected to an intermediate manifold 30a which in turn is connected to a main manifold 30b to which the gas mixture is delivered from a source of supply through a flexible conduit 31a. Although a single row of burners 28a is shown in Fig. 4, it should be understood that a plurality of rows of burners 28a may be provided, and that the number of burners and distribution thereof in the roof 23a is such that the desired heating effect may be produced in furnace chamber 29a.

The supply of gas mixture to each intermediate manifold 30a is controlled by a valve 32a, and the delivery of gas mixture to each burner is controlled by a member 33a which is associated with a valve (not shown) in the connection between the manifold 30a and the conduit leading to each individual burner.

In Fig. 4 the wire 10a to be annealed passes into a tube 60 at the charging end 25a of the furnace 15a. The tube 60 extends from the charging end 25a to the discharge end 27a of the furnace from which the annealed wire may pass into a quench tank and thence to a drying unit like those shown in Fig. 1, before being rewound. Although a single strand of wire is shown in Fig. 4, it is to be understood that in practice a plurality of strands of wire may be passed simultaneously through the furnace 15a alongside of each other and through tubes similar to the tube 60.

Immediately ahead of the charging end 25a of furnace 15a is provided a preheater or heating chamber 14a. The heating chamber 14a is similar to that in the embodiment first described and includes two banks of burners 45a similar to the burners 45. The burners 45a are mounted in and form a part of refractory walls 46a disposed within a framework or outer shell 47a. The burners 45a are connected to intermediate manifolds 48a which in turn are connected to a main manifold 49a to which a gas mixture is delivered through a flexible conduit 50a from a source of supply.

Although a single row of burners 45a is shown for each bank of burners in Fig. 4, it is to be understood that several rows of burners may be provided, as in the embodiment first described, and that each group of burners may be connected to an intermediate manifold 48a which in turn is connected to the main manifold 49. The supply of gas mixture to each intermediate manifold 48a is controlled by a valve 51a, and the delivery of gas to the individual burners is controlled by a member 52a which is associated with a valve (not shown) adjustable to control the supply of gas mixture to each individual burner.

In order to protect the wire 10a from burning in heating chamber 14a in the event of work stoppage, a housing 61 is secured to the shell 47a at the inlet side of the heating chamber. The housing 61 is formed to provide a plurality of spaced bearing surfaces 62 for supporting and guiding a movable annular sleeve 63. Under normal operating conditions the sleeve 63 is in

5 the position shown in Fig. 4. However, in the event of work stoppage, the sleeve 63 is moved into the interior of heating chamber 14a between the top and bottom burners 45a, thereby protecting the wire 10a from excessive heating.

In the embodiment of Fig. 4, the burners 45a are of a type capable of producing sources of radiant heat at temperatures varying from 2400 to 2800° F., thereby providing a preheater which will rapidly heat wires, strips and sheets and the like to an elevated annealing temperature, thereby permitting the furnace chamber 29a to serve as a holding and stabilizing chamber for its entire length. With this arrangement the work can be passed through furnace 15a at higher speeds than when introduced into the charging end of the annealing furnace without first being heated to the annealing temperature.

In view of the foregoing, it will be understood that I have provided an arrangement for heat treating work, such as sheets, strips, wires and the like, in which such work is held and maintained at a desired elevated temperature substantially during its entire travel through the heat treating furnace, thereby permitting the heat treating operation to be effected at relatively high speeds. While the supply of combustible fuel to the preheater may be immediately shut off in the event of work stoppage, it is nevertheless desirable to reduce the rate of heat input to the work when the rate of movement of the work decreases by either moving the burners 45 away from the work or by moving the sleeve 63 into the preheating chamber, as described above, because of the residual heat present at the refractory cupped burners embodied in the preheating chambers.

It may be desirable in some instances to effect annealing in the embodiment of Fig. 4 without the use of tubes through which the wires may pass, and in such case the burners 28a may be operated with a slight excess of gas to produce a reducing atmosphere. Although the annealing furnace 15a in Fig. 4 is provided with tubes, and such tubes are not shown in the embodiment illustrated in Fig. 1, it should be understood that tubes like tube 60 may also be provided in the furnace 15 of Fig. 1, if so desired. Further, when tubes like the tube 60 are employed, a suitable gas may be introduced into one end of the tubes to provide a protective atmosphere for the work passing through the tubes.

It has been previously pointed out that the work may be heat saturated in its entirety to a desired high temperature in the high heat capacity heating chamber, or that surface heat saturation may be effected with the inner core of the work heated to a desired high temperature requisite for the heat treating operation. In the claims, therefore, the words "heat saturated" should be interpreted to include either surface heat saturation of work or heat saturation of work in its entirety.

Although I have shown and described several 65 embodiments of my invention, therefore, such variations and modifications are contemplated as fall within the true spirit and scope of my invention, as pointed out in the following claims.

What is claimed is:

70 1. A method of heat treating which includes the steps of rapidly heating continuously metallic work of relatively long extent substantially to a desired elevated temperature by one or more relatively high temperature sources of heat in a place out of communication with a holding and

stabilizing chamber so that the work will be at the desired elevated temperature before it reaches the holding and stabilizing chamber, then passing said work through said holding and stabilizing chamber, and stabilizing said work substantially at said elevated temperature practically during its entire travel through said holding and stabilizing chamber, and reducing the heating effected by said high temperature source or sources of heat when the rate of movement of said work decreases to prevent overheating of the latter.

2. A method of annealing which includes the steps of rapidly heating continuously metallic work of relatively long extent substantially to an annealing temperature in a place out of communication with an annealing furnace by subjecting the strip to a temperature well above the annealing temperature so that the work will be at annealing temperature before it reaches said annealing furnace, immediately thereafter passing such work through said annealing furnace, holding said work substantially at the annealing temperature practically during its entire travel through said annealing furnace, and reducing the rate at which said work is heated prior to entering said furnace when the rate of movement of said work decreases.

3. A method of annealing which includes the steps of rapidly heating successive portions of metallic work of relatively long extent substantially to an annealing temperature in a place out of communication with a holding and stabilizing chamber by one or more relatively high temperature sources of heat, then passing said work through said holding and stabilizing chamber, maintaining said work substantially at the annealing temperature practically during its entire travel through said holding and stabilizing chamber, and moving said source or sources of heat in a direction from said work when the rate of movement of said work decreases.

4. Apparatus for heat treating continuous lengths of metallic work moving through a path at a high rate of speed including a heat treating furnace through which the work passes, an auxiliary heater through which said work passes before it reaches said furnace, said heater being formed of a plurality of parts located on opposite sides of the work as it moves through the path, means to heat said heater and furnace to impart heat to said work, said last-mentioned means being operative to supply a higher degree of heat to said heater than to said furnace, and means to move the parts of which said heater is formed away from the work to thereby prevent burning of the work, should its speed of movement be reduced.

5. Apparatus for heat treating continuous lengths of work moving through a path at a high rate of speed, an auxiliary heater located along said path, said heater comprising parts located on different sides of said work and movable relative to each other toward and from said work, a furnace surrounding said work and located in said path at a point beyond said heater, means located in the parts of said heater to produce a temperature sufficient to burn said work if it stopped moving to thereby rapidly raise the temperature of the work, means located in said furnace to maintain a given tem-

perature in said work substantially the same as that attained in said heater, and means to move the parts of said heater away from said work to thereby prevent burning of the same if said work should stop or slow down.

6. Apparatus for heat treating a continuous length of metallic work moving through a vertical path including a furnace having a chamber surrounding said work as it moves through said path, heating means located in said furnace to heat said work, tracks located on top of said furnace on opposite sides of said work at a point adjacent that at which said work enters said chamber, an auxiliary heater including parts mounted for movement on said tracks toward and away from said work, said parts cooperating to form a second chamber through which said work passes before it passes through said first-mentioned chamber, and means to move said parts along said tracks toward and from said work.

7. Apparatus for heat treating a continuous length of metallic work moving through a vertical path comprising a furnace having a chamber surrounding said work as it moves through said path, heating means located in said furnace to heat said work, an auxiliary heater mounted upon said furnace and having a chamber surrounding said work prior to the time it reaches said furnace chamber, said heater being formed of a plurality of separable parts located on opposite sides of said work, the chambers of said heater and said furnace being entirely separated, heating means located in the chamber of said heater operable to produce a higher thermal head than the heating means located in said furnace chamber, and means to move said parts of said heater toward and from said work to thereby vary the heating effect of said heater.

JAMES KNIVETON.

#### REFERENCES CITED

The following references are of record in the file of this patent:

#### UNITED STATES PATENTS

| Number    | Name           | Date           |
|-----------|----------------|----------------|
| 915,480   | Roberts        | Mar. 16, 1909  |
| 1,819,109 | Miller         | Aug. 18, 1931  |
| 1,890,065 | Meehan         | Dec. 6, 1932   |
| 1,956,401 | Russ           | Apr. 24, 1934  |
| 2,089,015 | Bucknam et al. | Aug. 3, 1937   |
| 2,136,957 | Sendzimir      | Nov. 15, 1938  |
| 2,162,692 | Baily          | June 20, 1939  |
| 2,200,732 | Woodson        | May 14, 1940   |
| 2,215,079 | Hess           | Sept. 17, 1940 |
| 2,261,702 | Tamele et al.  | Nov. 4, 1941   |
| 2,333,579 | Renkin         | Nov. 2, 1943   |

#### OTHER REFERENCES

Industrial Furnaces, vol. 1, 3rd edition, pp. 136, 137, 138, 189, and 190; edited by Trinks; published in 1934 by John Wiley and Sons, New York.

Making, Shaping, and Treating of Steel, 5th edition, pp. 1201 to 1204; published in 1940 by the Carnegie Illinois Steel Corporation, Pittsburgh, Pennsylvania.